

## UNITED STATES PATENT OFFICE

1,953,946

## METHOD OF AFFIXING STAMPS

Ernest B. Benger, Wilmington, Del., assignor to  
E. I. du Pont de Nemours & Company, Wil-  
mington, Del., a corporation of Delaware

No Drawing. Application October 17, 1931,  
Serial No. 569,535

38 Claims. (Cl. 216—62)

This invention relates to the uniting or affixing of gummed materials, such as labels, stamps, instruction sheets, price tags, trade-marks, etc., to materials which are normally non-responsive 5 to water-sensitive adhesives.

There are many materials, such as foodstuffs, chemicals, soap powders, tobacco and the like, which are susceptible to gain or loss of moisture. These materials are, preferably, packaged in a 10 material which prevents a change in moisture content.

Recently, there has appeared on the market a packaging material which is admirably suited for this purpose. It consists of a base combined, as 15 for example by being thinly coated on both sides, with a suitable moistureproofing composition. The base of the packaging material in its most common species consists of a sheet or film of regenerated cellulose, but it may consist of paper, 20 gelatin, metal foil, cellulose acetate and the like.

When the moistureproofing composition is applied to a transparent base, the product possesses a transparency which is at least equal to that of the base. In some cases, such as, for example, 25 when paper constitutes the base, the moisture-proof product is characterized by a transparency which is even greater than that possessed by the original base.

The moistureproofing composition contains a 30 waxy substance, and preferably a minor portion thereof. In its preferred form the moisture-proofing composition comprises a cellulose derivative, a gum or resin, a wax or wax-like material, with or without a plasticizer. In another form 35 the composition comprises a drying oil and a wax, while in the third modification it comprises a resin and a wax.

Recently it has become the vogue to wrap the 40 usual consumer cigarette package in a transparent moistureproof material, such as, for example, a moistureproof sheet or film of regenerated cellulose. A package so wrapped is not only rendered moistureproof and durable but also, due to the transparency of the wrapper, the legibility of 45 the printed indicia on the package is in nowise impaired.

Certain localities require a revenue stamp to be 50 affixed to the cigarette package by the retail merchant at the time of the sale. These stamps are usually gummed with a water-sensitive adhesive and, due to the fact that the surface of the moistureproof material is not responsive to such water-sensitive adhesives, it is impossible to affix the 55 stamp thereto by the common ordinary procedure, i. e., mere application of water to the adhesive.

Similarly it is impossible to affix other desirable 60 gummed devices, such as labels, instruction sheets, decorative stickers, etc., by moistening with water, to materials of the type hereinbefore

mentioned employed as wrappers or in any other way.

It has been found that by coating a predetermined area of a material which is normally non-responsive to water-sensitive adhesive with a composition comprising a gum, such as natural or synthetic rubber or the variants thereof, for example, 65 solutions and dispersions of caoutchouc, gutta percha, balata, rubber latex dispersions as well as solutions and dispersions of rubber-like substances, such as the polymers of isoprene, butadiene and their homologs, there will be provided 70 an area or zone which does not appreciably destroy the desirable properties of the material and to which devices, gummed with water-soluble adhesives, may be effectively affixed and secured by 75 merely superimposing the water-energized adhesive surface and applying sufficient pressure to bring the materials in intimate contact with each other.

It is therefore an object of this invention to provide a method of securing or affixing gummed materials to materials normally non-responsive to water-sensitive materials by providing a coating of a gum, such as natural or synthetic rubber 80 or the variants thereof, on a predetermined area of the material non-responsive to the water-sensitive adhesive, said coating being responsive to water-sensitive adhesives, whereby a water-energized adhesive superposed thereon will stick 85 thereto.

Another object of this invention is to provide 90 an article of manufacture comprising a material provided with a surface normally non-responsive to water-sensitive adhesive, for example, a moistureproof material such as a moistureproof sheet or film of regenerated cellulose, having a coating 95 which is responsive to energized water-sensitive adhesives and comprising a gum, such as natural or synthetic rubber or the variants thereof.

Additional objects will become apparent from 100 the following description and appended claims.

To explain the invention, it will be described in connection with wrappers, but as is obvious this is merely to illustrate one phase of the invention 105 and is not intended to restrict the invention there- to.

In accordance with the principles of this invention, a material which is normally non-responsive to water-sensitive adhesives and is to 110 constitute a wrapper is treated either before or after the contents have been packaged therein with a sizing composition which deposits a firmly adhering, and preferably also, flexible film or coating which is responsive to water-sensitive 115 adhesives. Preferably, the coating is deposited on a predetermined area of the wrapper where it is agreed that the gummed material is to be affixed.

The sized zone is not apparent to the layman. 120

It, however, can be detected by one skilled in the art because, due to the nature of the composition employed, the coating will be of very slight color, opacity, roughness or tackiness, not sufficient, however, to impair the appearance or serviceability of the wrapper. By virtue of the fact that the portion treated results from a coating, the essential characteristic of moistureproofness of the wrapper is not appreciably impaired. When the moistureproof wrapper is transparent, the film or coating applied may also be transparent with the result that this desirable characteristic is not impaired to any great extent. If desired, the coated areas may be made of a different hue or color and preferably harmonizing with the material packaged. This is accomplished by incorporating an appropriate coloring material, such as a dye or pigment, in the composition. In a like manner, by incorporating in the composition certain fillers or opacity-inducing agents, the film or coating may be made opaque.

The films or coatings, though sensitive to water-soluble adhesives, are devoid of any great degree of tackiness. This permits the piling, stacking or packaging of the coated materials or packages wherein the coated material constitutes the wrapper without the materials adhering to one another.

The sizing composition, which is employed in accordance with the principles of this invention, comprises a gum, such as natural or synthetic rubber or the variants thereof, for example, crepe rubber, gutta percha, balata, polymerized isoprene, butadiene polymers or the like, either alone or in combination with modifying agents, such as oils, resins, cellulose derivatives, softeners, casein, gelatin, metallic alkyl phthalates or the like dissolved, suspended or dispersed in a liquid vehicle. Preferably, the liquid medium is of low boiling point so that evaporation thereof may be obtained quickly. Toluene, benzene, carbon bisulfide and carbon tetrachloride, either alone or in combination, may be mentioned as a few of the numerous vehicles that have been successfully used. In some cases where for example the gum is used in combination with other substances, such as a cellulose derivative, and it is desired to dissolve the latter, the liquid vehicle may also contain a solvent for said cellulose derivative.

The proportions of the ingredients constituting the sizing composition may vary within wide limits. I have found that satisfactory results may be secured if the gum constitutes from 2%-20% or more of the final composition.

In order to more fully explain the invention, there is hereafter set forth several specific compositions which have given excellent results. It is to be understood that these examples merely illustrate a few of the numerous compositions which may be compounded and that they are not limitative of the invention:

Parts by weight

|                       |     |
|-----------------------|-----|
| 1. Gutta percha       | 10  |
| Toluene               | 90  |
| 2. Sheet balata       | 10  |
| Toluene               | 90  |
| 3. Deresinated balata | 10  |
| Benzene               | 90  |
| 4. Crepe rubber       | 98  |
| Carbon bisulfide      | 98  |
| 5. Oxidized rubber    | 10  |
| Carbon tetrachloride  | 90  |
| 6. Crepe rubber       | 19  |
| Glyptal resin         | 1   |
| Toluene               | 150 |

In compounding this composition the glyptal resin is rolled into the rubber mass in the well-known manner prior to the addition of the solvent. The glyptal resin, which is preferably used, is made by charging

80

|                     | Parts |
|---------------------|-------|
| Glycerin            | 14.6  |
| Phthalic anhydride  | 20.7  |
| Rosin               | 33.0  |
| China-wood oil acid | 31.0  |

85

into an open kettle and heating to a temperature of 250° C. over a period of two hours. The temperature is maintained at 250° C. for approximately six hours during which time a hot stream of carbon dioxide gas is bubbled through the mass or until the acid number is between 22 and 24.

90

If desired, suitable coloring agents, such as dyes or pigments, may be incorporated in the composition. Likewise, fillers and opacity-inducing agents may also be added.

95

The desired sizing composition is applied in any convenient manner to a predetermined area of, for example, a wrapping tissue of the type hereinbefore described. The solvent is then substantially eliminated by evaporation, preferably by heating, and the resulting material packed and packaged in the usual manner and shipped to the user. The wrapping tissue is finally enveloped about the article to be packaged. These wrapped packages are packed in the well-known manner, in which state they are distributed throughout the world.

100

When the usual consumer package of cigarettes is so wrapped, in those localities where a revenue stamp is required to be affixed by the retail merchant at the time of the sale, it is only necessary for the retail merchant to moisten a portion of the sized area and/or energize the water-soluble adhesive on the stamp with water, whereby upon superimposition of the stamp it may be readily affixed. The affixing is similar to the affixing of a postage stamp on an envelope or the like.

105

Instead of applying the coating to the wrapping tissue prior to the wrapping operation, the coating may be applied after the desired contents have been wrapped therein. For example, in the case of cigarettes, after the usual consumer package has been wrapped and sealed in the wrapping tissue the composition may be applied in any suitable manner to any predetermined portion of the package. Upon drying, the film responsive to the water-sensitive adhesive is formed. This package is then packed in cartons or the like and the stamp affixed, as previously described, at the time of the sale or at any other time.

110

Though the invention has been described specifically in connection with moistureproof sheets of films of regenerated cellulose, it is not restricted thereto since it is equally applicable to other materials non-responsive to water-soluble adhesives, such as, for example, moistureproof paper, moistureproof gelatine, pyroxylin objects, pyroxylin coated materials, synthetic plastic articles, cellulose acetate materials, and even to highly lacquered, varnished or painted materials, and metals or articles formed thereof, such as tin cans, foils, etc.

115

It is also to be understood that the invention is not restricted to the affixing of stamps, but that any gummed materials, such as labels, instruction sheets, trade-marks, etc., may be effectively affixed by utilizing the instant invention.

120

Though the preferred embodiment of the invention contemplates the affixing of devices gummed with water-sensitive adhesives to materials nor-

125

130

135

140

145

150

1 mally non-responsive to such water-sensitive adhesives, the invention is not limited thereto. The principles of the instant invention may be utilized in any process wherein it is desired to employ a 5 water-sensitive adhesive in conjunction with a material normally non-responsive to said water-sensitive adhesive. For example, a moistureproof material, such as a moistureproof sheet or film of regenerated cellulose, may be sized with one of 10 the compositions herein described on predetermined areas thereof, such as adjacent the edges thereof, and then upon the application of a water-sensitive adhesive the sheet may be sealed to itself. Such a procedure may be utilized in a process of 15 making tubes, bags, envelopes or the like. Likewise, two or more sheets may be secured together in the production of divers articles.

20 The terminology employed in the claims is intended to cover the material, either before or after it is enveloped about the contents packaged.

25 Since it is obvious that various changes may be made in the above description without departing from the nature and spirit thereof, this invention is not restricted thereto except as set forth in the appended claims.

I claim:

1. An article of manufacture comprising a material provided with a surface normally non-responsive to water-sensitive adhesives having a 30 coating comprising a gum of the class which consists of natural and synthetic rubber and the variants thereof responsive to water-sensitive adhesives, whereby devices gummed with water-sensitive adhesives may be affixed thereon.

35 2. An article of manufacture comprising a moisture-proof material normally non-responsive to water-sensitive adhesives having a coating comprising a gum of the class which consists of natural and synthetic rubber and the variants thereof on a predetermined area thereof responsive to water-sensitive adhesives, whereby devices gummed with water-sensitive adhesives may be affixed thereon.

40 3. A wrapping tissue comprising a transparent moistureproof material normally non-responsive to water-sensitive adhesives having a coating of a gum of the class which consists of natural and synthetic rubber and the variants thereof on a predetermined area thereof responsive to water-sensitive adhesives, whereby devices gummed with water-sensitive adhesives may be affixed thereon, the transparency and moistureproofness of said area not being destroyed.

45 4. A wrapping tissue comprising a transparent moistureproof material normally non-responsive to water-sensitive adhesives having a transparent coating comprising a gum of the class which consists of natural and synthetic rubber and the variants thereof on a predetermined area thereof responsive to water-sensitive adhesives, whereby devices gummed with water-sensitive adhesives may be affixed thereon.

50 5. An wrapping tissue comprising a moisture-proof sheet or film of regenerated cellulose having a predetermined area thereof coated with a gum of the class which consists of natural and synthetic rubber and the variants thereof, the moistureproofness of said area not being destroyed, whereby devices gummed with water-sensitive adhesives may be affixed thereon.

55 6. A wrapping tissue comprising a transparent sheet or film of regenerated cellulose having a transparent coating of a gum of the class which consists of natural and synthetic rubber and the variants thereof on a predetermined area thereof

responsive to water-sensitive adhesives, whereby devices gummed with water-sensitive adhesives may be affixed thereon.

7. An article of manufacture comprising a material provided with a surface normally non-responsive to water-sensitive adhesives having a coating comprising gutta percha responsive to water-sensitive adhesives, whereby devices gummed with water-sensitive adhesives may be affixed thereon. 80

85 8. An article of manufacture comprising a moistureproof material normally non-responsive to water-sensitive adhesives having a coating comprising gutta percha on a predetermined area thereof responsive to water-sensitive adhesives, whereby devices gummed with water-sensitive adhesives may be affixed thereon. 90

95 9. A wrapping tissue comprising a transparent moistureproof material normally non-responsive to water-sensitive adhesives having a coating of gutta percha on a predetermined area thereof responsive to water-sensitive adhesives, whereby devices gummed with water-sensitive adhesives may be affixed thereon, the transparency and moistureproofness of said area not being destroyed. 100

10. A wrapping tissue comprising a transparent moistureproof material normally non-responsive to water-sensitive adhesives having a transparent coating comprising gutta percha on a predetermined area thereof responsive to water-sensitive adhesives, whereby devices gummed with water-sensitive adhesives may be affixed thereon. 105

11. A wrapping tissue comprising a moisture-proof sheet or film of regenerated cellulose having a predetermined area thereof coated with gutta percha, whereby devices gummed with water-sensitive adhesives may be affixed thereon, the moistureproofness of said area not being destroyed. 110

115 12. A wrapping tissue comprising a transparent sheet or film of regenerated cellulose having a transparent coating of gutta percha on a predetermined area thereof responsive to water-sensitive adhesives, whereby devices gummed with water-sensitive adhesives may be affixed thereon. 120

125 13. An article of manufacture comprising a material provided with a surface normally non-responsive to water-sensitive adhesives having a coating comprising oxidized rubber responsive to water-sensitive adhesives, whereby devices gummed with water-sensitive adhesives may be affixed thereon.

130 14. An article of manufacture comprising a moistureproof material normally non-responsive to water-sensitive adhesives having a coating comprising oxidized rubber on a predetermined area thereof responsive to water-sensitive adhesives, whereby devices gummed with water-sensitive adhesives may be affixed thereon. 135

140 15. A wrapping tissue comprising a transparent moistureproof material normally non-responsive to water-sensitive adhesives having a coating of oxidized rubber on a predetermined area thereof responsive to water-sensitive adhesives, whereby devices gummed with water-sensitive adhesives may be affixed thereon, the transparency and moistureproofness of said area not being destroyed. 145

150 16. A wrapping tissue comprising a transparent moistureproof material normally non-responsive to water-sensitive adhesives having a transparent coating comprising oxidized rubber on a predetermined area thereof responsive to water-sensi-

- 5 tive adhesives, whereby devices gummed with wa-  
ter-sensitive adhesives may be affixed thereon.

17. A wrapping tissue comprising a moisture-  
proof sheet or film of regenerated cellulose hav-  
ing a predetermined area thereof coated with  
oxidized rubber, the moistureproofness of said  
area not being destroyed, whereby devices  
gummed with water-sensitive adhesives may be  
affixed thereon. 80

10 18. A wrapping tissue comprising a transparent  
sheet or film of regenerated cellulose having a  
transparent coating of oxidized rubber on a pre-  
determined area thereof responsive to water-sen-  
sitive adhesives, whereby devices gummed with  
15 water-sensitive adhesives may be affixed thereon. 85

19. An article of manufacture comprising a  
material provided with a surface normally non-  
responsive to water-sensitive adhesives having a  
20 coating comprising crepe rubber and a polyhydric  
alcohol-polybasic acid resin responsive to water-  
sensitive adhesives, whereby devices gummed with  
water-sensitive adhesives may be affixed thereon. 90

25 20. An article of manufacture comprising a  
moistureproof material normally non-responsive  
to water-sensitive adhesives having a coating  
25 comprising crepe rubber and a polyhydric al-  
cohol-polybasic acid resin on a predetermined  
area thereof responsive to water-sensitive adhe-  
sives, whereby devices gummed with water-sensi-  
tive adhesives may be affixed thereon. 100

30 21. A wrapping tissue comprising a transpar-  
ent moistureproof material normally non-respon-  
sive to water-sensitive adhesives having a coating  
35 of crepe rubber and a polyhydric alcohol-poly-  
basic acid resin on a predetermined area there-  
of responsive to water-sensitive adhesives, where-  
by devices gummed with water-sensitive adhe-  
sives may be affixed thereon, the transparency  
40 and moistureproofness of said area not being  
destroyed. 105

45 22. A wrapping tissue comprising a transparent  
moistureproof material normally non-responsive  
to water-sensitive adhesives having a transparent  
coating comprising crepe rubber and a polyhydric  
alcohol-polybasic acid resin on a predeter-  
50 mined area thereof responsive to water-sensitive  
adhesives, whereby devices gummed with water-  
sensitive adhesives may be affixed thereon. 110

55 23. A wrapping tissue comprising a moisture-  
proof sheet or film of regenerated cellulose hav-  
ing a predetermined area thereof coated with  
crepe rubber and a polyhydric alcohol-polybasic  
acid resin, whereby devices gummed with water-  
60 sensitive adhesives may be affixed thereon, the  
moistureproofness of said area not being de-  
stroyed. 115

65 24. A wrapping tissue comprising a transpar-  
ent sheet or film of regenerated cellulose having  
a transparent coating of crepe rubber and a poly-  
hydric alcohol-polybasic acid resin on a pre-  
determined area thereof responsive to water-sen-  
70 sitive adhesives, whereby devices gummed with  
water-sensitive adhesives may be affixed thereon. 120

75 25. A method of affixing devices, such as  
stamps, labels or the like, gummed with water-  
sensitive adhesives to a material having a sur-  
face non-responsive to water-sensitive adhesives  
which comprises applying a coating comprising  
80 a gum of the class which consists of natural and  
synthetic rubber and the variants thereof to a pre-  
determined area of said material, applying  
moisture to at least one of the surfaces of  
the materials to be disposed in contiguous rela-  
tionship and uniting the materials. 125

85 26. A method of affixing devices, such as  
stamps, labels or the like, gummed with water-  
sensitive adhesives to a transparent material hav-  
ing a surface non-responsive to water-sensitive  
adhesives which comprises applying a transparent  
coating comprising a gum of the class which con-  
sists of natural and synthetic rubber and the  
variants thereof to a predetermined area of said  
material, applying moisture to at least one of  
the surfaces of the materials to be disposed in  
contiguous relationship and uniting the mate-  
rials. 130

90 27. A method of affixing devices, such as stamps,  
labels or the like, gummed with water-sensitive  
adhesives to a material having a surface non-  
responsive to water-sensitive adhesives which  
comprises applying a composition comprising a  
volatile vehicle and a gum of the class which con-  
sists of natural and synthetic rubber and the  
variants thereof to a predetermined area of said  
material, evaporating the solvent, applying mois-  
ture to at least one of the surfaces of the mate-  
rials to be disposed in contiguous relationship and  
uniting the materials. 135

95 28. A method of affixing devices, such as  
stamps, labels or the like, gummed with water-  
sensitive adhesives to a material having a surface  
non-responsive to water-sensitive adhesives which  
comprises applying a composition comprising a  
volatile vehicle and 2% to 20% by weight of a gum  
of the class which consists of natural and synthetic  
rubber and the variants thereof to a predeter-  
mined area of said material, evaporating the sol-  
vent, applying moisture to at least one of the sur-  
faces of the materials to be disposed in contiguous  
relationship and uniting the materials. 140

100 29. A method of affixing devices, such as  
stamps, labels or the like, gummed with water-  
sensitive adhesives to a material having a sur-  
face non-responsive to water-sensitive adhesives  
which comprises applying a composition compris-  
ing a volatile vehicle and gutta percha to a pre-  
determined area of said material, evaporating the  
solvent, applying moisture to at least one of the  
surfaces of the materials to be disposed in con-  
tiguous relationship and uniting the materials. 145

105 30. A method of affixing devices, such as  
stamps, labels or the like, gummed with water-  
sensitive adhesives to a material having a surface  
non-responsive to water-sensitive adhesives which  
comprises applying a composition comprising a  
volatile vehicle and oxidized rubber to a predeter-  
mined area of said material, evaporating the sol-  
vent, applying moisture to at least one of the sur-  
faces of the materials to be disposed in contiguous  
relationship and uniting the materials. 150

110 31. A method of affixing devices, such as  
stamps, labels or the like, gummed with water-  
sensitive adhesives to a material having a surface  
non-responsive to water-sensitive adhesives which  
comprises applying a composition comprising a  
volatile vehicle, crepe rubber and a polyhydric  
alcohol-polybasic acid resin to a predetermined  
area of said material, evaporating the solvent, ap-  
plying moisture to at least one of the surfaces of  
the materials to be disposed in contiguous rela-  
tionship and uniting the materials. 155

115 32. A method of affixing devices, such as  
stamps, labels or the like, gummed with water-  
sensitive adhesives to a sheet or film of regenerated  
cellulose having a surface non-responsive to  
water-sensitive adhesives which comprises apply-  
ing a coating comprising a gum of the class which  
consists of natural and synthetic rubber and the  
variants thereof to a predetermined area of said  
sheet or film, applying moisture to at least one of  
the surfaces of the materials to be disposed in  
contiguous relationship and uniting the materials. 160

- the surfaces of the materials to be disposed in contiguous relationship and uniting the materials. 5
33. A method of affixing devices, such as stamps, labels or the like, gummed with water-sensitive adhesives to a transparent sheet or film of regenerated cellulose having a surface non-responsive to water-sensitive adhesives which comprises applying a transparent coating comprising a gum of the class which consists of natural and synthetic rubber and the variants thereof to a predetermined area of said sheet or film, applying moisture to at least one of the surfaces of the materials to be disposed in contiguous relationship and uniting the materials. 10
- 15 34. A method of affixing devices, such as stamps, labels or the like, gummed with water-sensitive adhesives to a sheet or film of regenerated cellulose having a surface non-responsive to water-sensitive adhesives which comprises applying a composition comprising a volatile vehicle and a gum of the class which consists of natural and synthetic rubber and the variants thereof to a predetermined area of said sheet or film, evaporating the solvent, applying moisture to at least one of the surfaces of the materials to be disposed in contiguous relationship and uniting the materials. 20
- 25 35. A method of affixing devices, such as stamps, labels or the like, gummed with water-sensitive adhesives to a sheet or film of regenerated cellulose having a surface non-responsive to water-sensitive adhesives which comprises applying a composition comprising a volatile vehicle and 2% to 20% by weight of a gum of the class which consists of natural and synthetic rubber and the variants thereof to a predetermined area of said sheet or film, evaporating the solvent, applying moisture to at least one of the surfaces of the materials to be disposed in contiguous relationship and uniting the materials. 30
- 40
- 45
- 50
- 55
- 60
- 65
- 70
- 75
- surfaces of the materials to be disposed in contiguous relationship and uniting the materials. 36. A method of affixing devices, such as stamps, labels or the like, gummed with water-sensitive adhesives to a sheet or film of regenerated cellulose having a surface non-responsive to water-sensitive adhesives which comprises applying a composition comprising a volatile vehicle and gutta percha to a predetermined area of said sheet or film, evaporating the solvent, applying moisture to at least one of the surfaces of the materials to be disposed in contiguous relationship and uniting the materials. 80
- 85
- 90
- 95
- 100
- 105
- 110
- 115
- 120
- 125
- 135
- 140
- 145
- 150
- ERNEST B. BENGEL.